

[54] PRESSURE SENSITIVE RESISTANCE AND  
PROCESS OF MAKING SAME[75] Inventor: Michael Michalchik, Newport  
Beach, Calif.[73] Assignee: Dynacon Industries, Inc., West  
Milford, N.Y.

[21] Appl. No.: 575,184

[22] Filed: May 7, 1975

## Related U.S. Application Data

[63] Continuation-in-part of Ser. No. 335,499, Feb. 26, 1973,  
abandoned.[51] Int. Cl.<sup>2</sup> ..... H01B 1/02[52] U.S. Cl. ..... 252/512; 252/511;  
252/513; 252/514; 338/114[58] Field of Search ..... 252/511, 512, 513, 514;  
260/37 M; 428/403; 338/114

## [36] References Cited

## U.S. PATENT DOCUMENTS

3,281,403 10/1966 Manuel ..... 252/513 X  
3,359,145 12/1967 Salyer et al. ..... 252/5133,469,441 9/1969 Pohl ..... 252/500 X  
3,629,774 12/1971 Crites ..... 338/114  
3,709,835 1/1973 Forster ..... 252/513 X  
Re. 28,595 10/1975 DuRocher ..... 338/114 X

Primary Examiner—Richard E. Schafer

Assistant Examiner—E. Suzanne Parr

Attorney, Agent, or Firm—Frank L. Durr; Orville N.  
Greene

[57]

## ABSTRACT

A pressure sensitive resistance material and process for making the same is described which is of the type comprising an elastomeric matrix with conducting metal particles dispersed therein. Improved performance and improved ranges of conductivity between the no pressure and pressure ranges are obtained by coating the metallic conducting particles with semi-conducting material and further improved results are obtained when the semi-conducting material comprises a reaction product of an organic metal compound with an aryl peroxide of similar aryl compound. The material may be made available as a coating material or as a shaped product.

18 Claims, 1 Drawing Figure





## PRESSURE SENSITIVE RESISTANCE AND PROCESS OF MAKING SAME

This application is a continuation-in-part of application Serial No. 335,499 filed February 26, 1973 now 5 abandoned.

According to said prior application, improved pressure sensitive resistance material of the type containing metal conducting particles embedded in an elastomeric matrix, have been obtained when the metal particles are pretreated with a organic compound (which in some cases acts as an inhibitor of catalysis or the matrix material). Further improved results were obtained by reacting the coated metal particles with an aryl type of peroxide. It has also been found that the reaction of organic metallic compounds with peroxides, especially aryl peroxides, can be prepared and then applied to the metal particles with the aid of a solvent. Also, additional semi-conducting compounds and additional matrix materials not disclosed in said original application, have been found to produce equivalent desired results. In addition, it has been found that the original range of the amount of the coating material was erroneously set forth in the prior disclosure.

This invention relates to pressure sensitive resistance elements and to process of producing the same. The pressure sensitive resistance material may also be in the form of a plastic composition and applied as a coating.

Pressure sensitive resistance devices are well-known. Generally, such devices comprise a matrix of insulating, elastomeric or yieldable material in which is dispersed, more or less uniformly, a multiplicity of relatively fine, electrically conducting powders. The following conducting particles have been suggested for embedding in a non-conducting matrix, although not always for a 35 pressure sensitive product, iron, copper, chromium, titanium tungsten, platinum, boron, stainless steel, silicon, silver, gold, nickel, cobalt, aluminum, zinc, "Ni-chrome," carbon (in the form of carbon black or graphite, for example), etc. The metals or carbon may be in the form of strands, flakes, spheres or irregularly shaped particles and the sizes of the metal particles, which have been specified as useful, may vary from about 0.003 microns up to about 100 mils (2500 microns) although it is generally agreed that smaller particles are preferred; also, with respect to carbon additions, some exceptionally finely divided carbon materials have been employed.

Among the objects of the present invention is to provide a pressure sensitive material or element of the type 50 wherein small conducting metallic particles are embedded in a flexible or elastomeric base, which element is normally of high resistance but has a very low resistance under pressure.

Among other objects of the invention is to provide a 55 pressure sensitive switching material or element of the type described which repeatedly and substantially uniformly, under pressure, changes from an insulator of high resistance to a low resistance conductor.

Among still further objects of the invention is to provide a pressure sensitive element of the type described which has transducer properties in that it has a substantial region where the conductance thereof varies directly with the pressure applied as approximately a straight line or predictable function.

Among still further objects of the invention is to provide a pressure sensitive resistance material or element of the type described which has a greater range of

change in resistance and is responsive to smaller forces than heretofore possible.

The objects of the invention are attained by coating metallic conducting particles with a deformable, semi-conducting coating material and incorporating the coated particles in a suitable elastomeric matrix. Preferably, the conducting particles are pretreated with a solution containing the deformable, semi-conducting or potential semi-conducting material before being added to the matrix-forming resin composition. The potential semi-conducting material may be of such a nature as to inhibit polymerization of the resin composition and this also may be advantageous in that the polymerization of the resin is inhibited only at the interfacial region between the individual conducting particles (or the coating thereon) and the matrix. Thus, the conventional process of preparing such products is to add the clean conducting metallic particles and a polymerizing catalyst or vulcanizing agent to the monomer (or partially polymerized) elastomeric composition which is to form the matrix, then casting or molding the mix and curing it to form the polymerized or vulcanized product. According to the present invention, the conventional process or composition is modified so as to include a deformable substance which is adsorbed on the particles, which act to facilitate the conduction of electricity between the particles when the matrix is compressed or stretched to bring adjacent particles closer together, and which may also inhibit or alter the curing of the matrix material.

A practical way for carrying out the process is to prepare the deformable semi-conducting material (instead of forming it in situ on the metal particles) and then applying it to the metal particles, as necessary, before mixing with the matrix material, by for example, dissolving in a solvent and applying to the metal particles. The term deformable, semi-conducting material, as used in this specification and claims will be understood to include non-liquid, organic or inorganic semi-conducting materials which are in a condition to coat the metallic particles, either directly or from solution in a solvent and which have resistivities of  $10^{-2}$  to  $10^7$  ohm centimeters.

The metallic conducting particles added can be any of the metallic particles mentioned above with respect to the prior art. It is found, however, that particles having large specific surface areas produce the best results. Raney nickel is a commercially available material of relatively high specific surface area and produces very good results as does the nickel known on the market as carbonyl nickel (precipitated from nickel carbonyl). Where it is desired that a circuit cease operating after a certain time (for example, after 10-45 days), mercury coated nickel particles can be employed. The size of the metallic conducting particles preferably varies from about 0.1 to about 44 microns, or (preferably) pass a 325 mesh screen.

In addition to those metals mentioned in the prior art, metal particles not heretofore useful in the production of such pressure sensitive resistances, can be employed by the present invention. Thus, aluminum particles when coated according to the invention and dispersed in an elastomeric matrix, produce a pressure sensitive conductor in spite of the fact that aluminum is known to form a passive, non-conducting, metal oxide surface almost instantly in the presence of air. Actually, the carbonyl nickel particles which have been coated according to this invention, are also more conductive than

the uncoated particles, although the change in conductivity is not as dramatic as with aluminum particles

The ratio of elastomeric resin to conducting particles can vary from about 100:75 to 100:110 by weight. A very satisfactory product has a ratio of resin to conducting particles as set forth above and metal conducting particles of a size below 3 microns with a surface area of about 0.5 m<sup>2</sup>/gram or more. However a greater reproducible switching effect occurs when there is a mixture of larger spherical particles with the smaller particles, e.g., 75 vol. % of particles 0.2-0.5 microns plus 25% of spherical particles of 5-7 microns in diameter.

Silicone elastomers are one preferred matrix material since these products have good insulating and other electrical properties, retain their basic physical properties over a wide range of temperature, are inert and oxidation resistant with respect to the atmosphere, are inert and corrosion resistant with respect to most chemicals and are water repellent and resist weathering. Among the silicone elastomeric compositions available commercially, the "RTV" (room temperature vulcanizing) type are suitable and preferred because of the ease in carrying out the vulcanization or polymerization or cross-linking. At least two types of such RTV silicone resin compositions are available, one of which is essentially a heat curing silicone in which the curing reaction is promoted by the addition of a peroxide curing agent and one in which the curing is promoted by the addition of metal soap (especially tin and cobalt soaps). Although said two types of compositions produce polymerized or vulcanized elastomers of substantially the same chemical structure (i.e. long chain structures of the general formula



where R is usually a lower alkyl radical, with cross-links between the chains), the soap type of polymerizable composition is usually incompatible with the peroxide type and the catalyst useful for the soap type of composition (i.e., a metal soap) usually acts as an inhibitor to polymerization in the peroxide type of composition and vice versa. According to the present invention, the semi-conducting coating material which is added to the composition, or preferably to the conducting particles in a pretreatment step, may also be an inhibitor to the polymerization of the resin. Silicon compositions which contain fillers such as silica, asbestos, mica, etc., which increase the viscosity of the unpolymerized composition are also useful in this process.

Although silicone compositions are the preferred type of matrix-forming compositions, other flexible or elastomeric-producing, monomeric or flowable intermediate polymeric compositions may be employed as matrix forming materials. Such compositions are widely available commercially and include the natural and synthetic rubbers, polymerizable urethanes, polyalkylenes, ethyl vinyl acetate, polyvinylchloride, etc. However, with natural and synthetic rubbers, sulfur should be excluded as the vulcanizing agent.

In addition, polymerizable or resin-forming mixes may be partially polymerized or thickened to a degree just sufficient to form a more or less adhesive liquid composition and mixed with the electrically conducting coated metal particles described herein, to provide a marketable flowable adhesive composition useful for

forming electrically conducting coatings on various substrates.

Suitable catalysts for the peroxide type of silicone elastomers include tert-butyl peroxyphthalate, 2,4-dichlorobenzol peroxide, caproyl peroxide, lauryl peroxide, p-chlorobenzoyl peroxide, tert-butyl peroxyisobutyryle, acetyl peroxide, benzol peroxide, di-tert-butyl diperphthalate, tert-butyl peracetate, tert-butyl perbenzoate, dicumyl peroxide, 2,5-dimethyl-2, 5-di(tertbutyl peroxy) hexane, di-tert-butyl peroxide, methyl ethyl ketone peroxide, p-methane hydroperoxide, cumene hydroperoxide, tert-butyl hydroperoxide, etc. Such catalysts can be used alone or in combination or in solution in a suitable solvent. It appears that a trace of aluminum powder or contact of the metallic particles with an aluminum surface improves the formation of the resistance materials of this invention.

The deformable, coating material for the metal particles can be a material which has semi-conducting properties or one which, by reaction with other material in the mix (the peroxide catalysts, for example), results in a deformable, conducting material and it may include a portion of the elastomeric composition from which the matrix is to be formed. In many of the examples which follow the semi-conducting material is the reaction product of a tin or lead soap with a peroxide because that was the way by which the effect was discovered. Suitable metal soaps for this type include tin laurate, dibutyl tin diluariate, stannous octoate, cobalt octoate, lead octoate, lead naphthenate and similar nickel, manganese and molybdenum soaps. The reaction of such soaps with the peroxides mentioned in the previous paragraph provides a very desirable semi-conducting material and resembles an inorganic polymer; preferably the reaction is carried out in the presence of an aryl compound if the peroxide itself does not contain an aryl group. As already mentioned above, the process is simplified when the metal soap and peroxide (preferably aryl peroxide) are prereacted to provide a compound which can be later applied to the metal particles. It is believed that some such reaction products comprise a polymer with (-O-Sn-O-Sn-O) bonds (where tin soap is employed) since the reaction products gradually thicken and have film-forming properties. The conductivity of a stannic oxide-aromatics junction has already been described by H. Inokuchi et al (from the test: Symposium on Electrical Conductivity in Organic Solids—Office of the Ordinance Research, Duke Univ., Durham, N.C., Apr. 20, 22, 1960. Interscience Publishers; see chapter, "The Photovoltaic Behaviors of Aromatic Hydrocarbons"). Also, the many metal complexes which have semiconducting properties are useful in this invention, see "Organic Semi-Conductors" by Okamoto and Walter Brenner, New York University, Reinhold Publishing Corp., 1964, pages 66-68. In addition, the non-metallic, complex semi-conductors such as the semi-quinone type molecular complexes disclosed on pages 69-71 of the same references can be employed. In this connection, it is noted that U.S. Pat. No. 3,469,441 discloses a quinone type polymer which per se, acts as a pressure sensitive resistance.

According to the present invention, the amount of the organic conducting material added to the conducting powder can vary from about 5% (based on the weight of the powder) down to about 0.02%.

As already indicated, semi-conducting materials which inhibit curing of a resin, or which comprise com-

## EXAMPLE IA

ponents or reaction products which inhibit curing, may be employed and have appeared to enhance the effect desired. Thus, the metal soaps may inhibit curing of the peroxide cured silicone resins at interfacial zones between the metal particles and the resin matrix. In some cases also, water, a polymerization inhibitor, may be added to form a slurry of the metal powder prior to mixing with the resin forming matrix material.

In a preferred form of the invention, the metal conducting particles are coated with the deformable, semi-conducting coating material prior to adding to the elastomeric, matrix-forming, material and the semi-conducting material is a complex type of compound such as one having charge transfer properties or a metallo organic type of complex. The coating appears to form a boundary area or separate phase between the metal particles and the matrix resin. In the cases where the coating layer is an inhibitor of polymerization, it is believed that the inhibited polymerization product is more adherent to the metal particles than the bulk of the polymerized matrix. It has been discovered, however, that the effects in the finished product can be destroyed by severe hammering and this result is attributed to the removal or destruction of the coating. Another explanation of the destruction of the effects by hammering is that the coated particles form agglomerates which are loosely connected even after thorough mixing with the matrix.

The products of the invention show appreciable decrease in resistance when placed under tension, as well as when compressed.

The FIGURE in the drawing is a resistance-pressure curve shown by one of the products.

The invention will be exemplified in the following specific examples with the understanding that these examples are preferential and illustrative and not be considered as limiting the invention to the date given.

## EXAMPLE I

Ten grams of silicone resin composition known as RTV-11 (an RTV resin polymerized with the aid of a metal soap and sold by General Electric) was combined with 2 drops of tin octoate and 2 drops of 60% methyl ethyl ketone peroxide dissolved in dibutyl phthalate. As soon as these materials were thoroughly mixed, 8 grams of the slurry of Raney nickel were added and thoroughly mixed. The Raney nickel, which is a very finely divided nickel that is pyrophoric, was made into a slurry with an organic liquid such as an alcohol, replacing water. The 8 g of slurry added was largely nickel, but included the weight of the organic liquid. The mix was doctored into molds to a thickness of 1/16 to 1/2 inch, allowed to set at room temperature for 45 minutes and gradually heated to 105° C., over a period of 1 hour, and then maintained above 100° C for 20 minutes. The resultant strip, about 0.200 inches thick, showed a resistance between electrodes, 1/6 inch round probes on opposite sides of the strip, of from 10 meg-ohms under no pressure, down to 1000 ohms under manually applied pressures. Unless otherwise specified, all tests recorded below were made by these same probes and a resistance meter. The repeatability of resistance under a given compressive force was found to be within 5%. When the strip was cut and trimmed, improved results were obtained and the improved results were attributed to the improved configuration of the resistance element between the electrodes.

- 10 Two drops of stannous octoate, 2 drops of dibutyl tin laurate and 0.1 g of benzoyl peroxide were dissolved in 6 g of benzene and the solution mixed with 10 g of silicone resin, GE's RTV 11. After thoroughly mixing with the aid of a spatula, a slurry containing 8 g of nickel powder (a carbonyl nickel powder sold by Internation Nickel company and identified as Mond 255) was added and mixed therewith. The Mond 255 nickel has a specific surface of about 0.5 m<sup>2</sup>/g. The slurry was made with 4 grams of water, all of the excess water having been pressed out of the cake. The mixture with excess solvent was thickened by evaporation and cast onto an aluminum foil and allowed to remain overnight. The resultant set mixture was baked for 3 hours at 110° C.
- 15 20 In Sections 20 mils thick, the resistance between probes was changed from 500 ohms to 2 ohms under pressure.

## EXAMPLE 2

- 25 30 Two drops of stannous octoate, 2 drops of dibutyl tin laurate and 0.1 g of benzoyl peroxide were dissolved in 6 g of benzene and the solution mixed with 10 g of silicone resin, GE's RTV 11. After thoroughly mixing with the aid of a spatula, a slurry containing 8 g of nickel powder (a carbonyl nickel powder sold by Internation Nickel company and identified as Mond 255) was added and mixed therewith. The Mond 255 nickel has a specific surface of about 0.5 m<sup>2</sup>/g. The slurry was made with 4 grams of water, all of the excess water having been pressed out of the cake. The mixture with excess solvent was thickened by evaporation and cast onto an aluminum foil and allowed to remain overnight. The resultant set mixture was baked for 3 hours at 110° C.
- 35 40 In Sections 20 mils thick, the resistance between probes was changed from 500 ohms to 2 ohms under pressure.

## EXAMPLE 2A

- 45 50 Example 2 was repeated with 7 grams of water added to the nickel powder to form a wet slurry which exudes a few drops of water when mixed with silicone.

Areas of the material showed switching action between 200 k ohm to 50 ohm under probe pressures. In one section, 1/4 inch thick, the material switched from near open circuit under no pressure down to 200 ohms under repeated pressure.

The materials of Example 2 adhered rather well to aluminum.

- 55 60 The above examples were not the best samples prepared according to the invention, but were sufficiently improved over products familiar to inventor to lead the way to further improvements. It will be noted, for example, that although the resin composition RTV 11 of General Electric, employed in Examples 1-2A is a resin which is adapted to be set by a metal soap, these examples included a peroxide catalyst which ordinarily inhibits polymerization of these resins. Examples 2 and 2A also employ an aqueous slurry of the metal particles and water is also known as an inhibitor. The following examples show later developments of the invention.

## EXAMPLE 3

- 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505

ing between 1 and 1.5 meg-ohm down to 3 ohm (under pressure) were obtained.

#### EXAMPLE 4

90 g of Mond 255 nickel powder was introduced into a solution of 1 g of tin octoate in 20 g of tetrachlorethylene and allowed to stand for several hours at room temperatures. In a separate vessel 90 g of Dow RTV 3120 silicone resin (a tin soap catalyzed type of silicone composition which contains iron oxide filler and has a pasty consistency) was mixed with a solution containing 9 drops of tert-butyl perbenzoate in 20 g of ethyl alcohol and the mixture was degassed (by applying a vacuum, for example). Excess liquid was decanted from the metal slurry and the remaining slurry mixed with the resin, and the mix poured into a pan mold. The mold was heated slowly to 95° C. and maintained at this temperature for a period of 1 hour whereupon some evaporation and some curing took place. The tacky mixture was allowed to stand at room temperature for 24 hours. Final curing was carried out at 150° C. Strips from about 1/32 to  $\frac{1}{8}$  inches thick showed resistances through the thickness varying from 100,000 ohm under no pressure to less than 1 ohm under pressure.

#### EXAMPLE 5

100 g of nickel powder (Mond 255) was mixed with a solution of 2 g of tin octoate in 20 g of butanol and the mix allowed to stand for several hours. In a separate vessel, 100 g of the silicone resin composition GE RTV 560 (a metal soap catalyzed type of polymerizable resin) was mixed with a solution of 0.5 g of tin laurate and 9 drops of tert-butyl perbenzoate in 20 g of butanol. The resin solution was mixed with the metal slurry, the mix deaerated and cast into two pans, one of which was covered and the other left uncovered. The cure of the mix of the covered pan was inhibited. Both pans were cured as in Example 4. The resultant cured sheets gave a switching action type of product having a resistance between 10,000 ohms at no pressure to about 0.20 ohms under pressure with different pressure sensitivities for the differently formed sheets (better sensitivity in the inhibited sheet).

#### EXAMPLE 6

In a mix of 1 g tin octoate, 40 g of perchloroethylene and 10 drops of tert-butyl peroxybenzoate, 97 g of carbonyl nickel powder was dispersed and the mix gently heated to about 110° C. in a loosely closed container for about 1 hour. In a separate vessel, 102 g of the silicone resin composition GE RTV 21 (a metal soap polymerizing composition) and 0.5 g of dibutyl tin laurate were mixed and degassed. After cooling, the nickel powder with the remaining perchloroethylene was mixed with the resin, cast to form a strip and cured 2 hours at 80°. The cured strip was about 1/16 inches thick and functioned exceptionally well as a switching action type of resistance having a resistance of 1 megohm under no pressure down to 10 ohm under manually applied pressure between electrodes of the resistance meter.

#### EXAMPLE 7

The process of Example 6 was repeated substituting another soap cured silicone resin, namely GE's RTV 560, for the RTV 21 and increasing the Ni:Resin ratio to 1:1. The product obtained had a resistance range from less than 1 ohm to 1 megohm and had a diode effect.

The diode or pressure polarizable effect referred to above was discovered on a 1/16 inch thick material subjected to 10-15 cycles per minute at 12-15 psi and 5 volts with a 1100 ohm limiting resistance in series.

5 Under these conditions, the material showed a gradual decay in conductivity over a period of 5-15 minutes from a resistance in the low range of less than 1 K to over 100 K with the high end remaining over 100 k. Reversing polarity in the specimen between the silver electrodes produced instant return response with the low values below 1 k Ohm. The mechanical strength remained constant. The electrical effect progresses under cycling even when the current is interrupted.

10 Pressure polarizable products such as disclosed in Example 7 are useful as passive counting materials, flexible electromechanical memory sensors, persistent display and readout devices which are erasable by electrical polarity switching, pacing and recycling aids in teaching machines, low cycle randomizing actuators and such other applications where properties of persistence are uniquely cumulative so that energy input, work expended, time, force and voltage vectors can be recorded. Thus simplified, bio-feedback circuitry and instrumentation devices, which have memory within 15 the sensor element are made possible.

20 The procedure of Examples 1-7 has been followed to produce products in which the conducting metal is a silver, tin, copper, silver coated nickel, and mercury coated nickel. With the mercury coated nickel, the product showed a range of resistance of 1 ohm to 1 meg, but then, after a period of about 10-45 days, showed a resistance of 1000 ohms under pressure. When carbon is added to any of the above Examples, it apparently absorbs catalyst from the resin and a long period of cure is 25 required.

#### EXAMPLE 8

30 The same procedure as in Example 6 has been employed with a foaming type of silicone resin, GE's RTV 7, which has cured with dibutyl tin laurate, the nickel particles being pretreated as in Example 6. The curing of the resin was inhibited by the peroxide coated nickel, but the forming proceeds and after an additional curing for about two weeks at room temperature, a  $\frac{1}{8}$  inch 35 thick, non-sticky tape was obtained which had a transducer action in a low range of resistance from 25 ohms at 60 psi to 4 ohms at 105 psi.

#### EXAMPLE 9

50 A mixture of 10 g stannous octoate, 3.3 g of butyl-peroxybenzoate in 10 g of perchloroethylene was allowed to react slowly without gassing and then heated to 95° C for 30 minutes and allowed to cool. 100 g of Mond 255 nickel was treated with 1.5 g of the resultant mix, the solvent removed and the metal dried.

55 A second additive was prepared adding 10 g of chloral to 30 g of stannous octoate and then adding 10 g of tertbutylperoxy benzoate. Heat was evolved during these additions. 0.5 g of this second additive was added to the 6.3 g of the polyol portion of a two component polyurethane resin. In such polyurethane compositions, one component is a polyisocyanate and one is a polyol in the mol proportions of approximately 2:1. The resin component employed was the Polycin 879 of Baker Castor Oil Co. 15 g of the nickel mix above was added to the Polycin 879 and then 3.7 of the polyisocyanate, Vorite 689 M-2 (also of Baker Castor Oil Co.), was added. The mix was cast on aluminum foil heated to 90°

C to initiate the cure and then allowed to complete the cure at room temperature for 10 hours. Thereafter, the mix was finally cured at 90° for 30 minutes to provide a flexible film 1/16 inch thick. The film had a resistance of 100 ohm at no pressure to 6 ohms with hand applied pressure between the electrodes.

The following Example discloses the idea of prereacting the metal organic compound with a complex forming reagent such as the aryl peroxides.

#### EXAMPLE 10

Two grams of tin octoate and one gram of 1, 1-di-t-butyl peroxy-3,3,5-trimethylcyclohexane (a peroxy catalyst supplied by Noury Chemical Co.), were diluted with a little trichlorethylene and allowed to heat to about 200° C. After a brisk, smoky reaction, taking about 5 minutes, one gram of the resultant viscous, product was dissolved in dichlorethane, 50g, and mixed thoroughly with 100 grams of Mond Nickel Powder 225, then thoroughly dried by heating to 120° in an oven, and then mixed with an equal amount of GE's RTV #21. To the mixture 0.5 of a catalyst, dibutyl tin dilaurate, was added and the mix cast and cured to form a thin film 1-2 mm thick. The film produced had a resistance varying from 5-10 megohms under no pressure, down to 5-10 ohms under firm pressure.

In the above Example, the reproducability of the resistance under fixed pressure could be increased by replacing the 100 g of Mond Ni with 100 g of a mix containing 75 vol % of Mond nickel and 25 vol % of small nickel spheres of 5-7 microns in diameter.

Similar reaction products of the following metal organic compounds: dibutyl tin hexoate, stannous oleate, manganese octoate, dibutyl tin oxide, dibutyl tin dichloride, tetraphenyl tin, nickel caprylate, cobalt octoate, germanium tetraethyl and lead octoate; were treated with one or more of the following peroxides: (a) tert-butyl peroxybenzoate (b) 1,1-di-t-butyl peroxy-3,3,5-trimethylcyclohexane (Percadox 29-c-75), (c)  $\alpha$ ,  $\alpha$ -bis(t-butyl peroxy) diisopropyl benzene (Percadox 14); in the ratio of two parts of the metal compound to one part of the peroxide. In all cases, a reaction occurred and a film-forming product was produced which dissolved in trichlorethylene. When such reaction products were applied as a coating to Mond Nickel Powder 255, and the powder was subsequently mixed with a substantially equal weight of silicone resin composition, cast films therefrom showed pressure sensitive resistance properties varying from the order of 10 megohms under no pressure to the order of 1 ohm under pressure.

The following Example discloses that the process is effective with aluminum powder in spite of the fact that aluminum, exposed to air, is known to have a passive oxide coating thereon.

#### EXAMPLE 11

A reaction product similar to that of Example 10 was formed between 2 parts of nickel acetoacetone and one part of 1,1-di-t-butyl-peroxy-3,3,5-trimethylcyclohexane. One part of the reaction product dissolved in acetone was applied to 100 parts of finely divided aluminum powder (Alcan MD 294) and the mix dried at 120° for 1 hour. The resultant material was sieved and the appearance thereof was practically the same as the original Al powder. Thereafter, 50 grams of the powder were mixed with 50 g of silicone resin composition (#21 RTV of General Electric), 25 g of benzol was added as a thinner and 6 drops of dibutyl tin laurate added as a

catalyst. The mix was degassed and cast to the form of a film. The set film was still somewhat bubbly and showed a resistance of the order of 1000 megohms under no pressure, but a resistance of several ohms under pressure.

Absent the coating on the Al powder, it has not been possible to make a pressure sensitive film with any degree of conductivity under pressure, and, in fact, it has been found impossible to take flakes of Al and compress them between electrodes so as to obtain any degree of conductivity.

It is not necessary that the conductive coating material for the metal particles include a radical resulting from reaction with a peroxy compound. The following Examples 12-13 show alternative reaction products.

#### EXAMPLE 12

1 g of glycerophosphoric acid was dissolved in 50 ml of tetrahydrofuran. The mixture was added to 100 g of finely divided Ni powder (Carbonyl Ni), and the slurry heated to a fairly high temperature of 160° to vaporize the solvent and to provide a residue-covered Ni powder. The coated powder was dispersed in 90 g of silicone resin composition (RTV-11 of General Electric) to which 1 g of manganese octoate catalyst had been added just prior to adding the metal. The mix was cast and cured at 100° C for 3 hours, then post cured at 135° C for 1 hour.

The product had a resistance under no pressure of 10 megohm and a resistance under manually applied pressure of 20 ohms.

The coating material of Example 12 is especially suitable when the matrix material is to be made from a solution of the silicone resin since this coating is not soluble in hexane or benzene which are the usual solvents used to dilute or dissolve the resin. Some instances of non-uniform results have been traced to a dissolution of the coating by the solvent for the elastomeric matrix material.

#### EXAMPLE 13

0.9 g of tin poly (cobaltinum esters), (Abstract No. 68 of the Industrial and Engineering Chemistry Division of A.C.S. for the Chicago meeting, Aug. 27-31, 1973, discloses a method of making such esters), was dissolved in 300 ml. of benzene at refluxing temperature. 100 g of finely divided Nickel Powder (Mond 255) was rapidly added to the sealed refluxing solution while stirring and the refluxing continued for 4 hours at the boiling temperature. The treated metal was filtered and allowed to dry in an inert nitrogen atmosphere. 90 g of a silicone resin composition (RTV-11) to which 0.5 g of dibutyl tin laurate was added, was degassed and then carefully mixed with the treated nickel powder. The mix was cast and allowed to harden at 90° then post cured at 120° overnight. The resulting product had a resistance of 100 K ohms under no pressure and a resistance of 0.1 ohms under manually applied pressure.

The tin poly (cobaltinum ester) of Example 13 is one of a group of metallocene compounds which are film forming, charge transfer type complexes and show semi-conductor properties so as to be suitable for coating the metal conducting powders of the present invention. The theoretical aspect of conductivity in charge transfer complexes is given in the Review of Published Data, published by John Wiley & Sons, Inc., in Organic Semiconductors (Felix Gutmann and Lawrence E. Lyons), 1967, Section 8.4, pp b 460-463 (the last complete

paragraph on page 462 states that "the resistivity minimum is most pronounced in the strongly interacting complexes," etc.).

As already mentioned, silicon resins are a preferred matrix material although other elastomeric resins may be employed. A portion of the desirable properties obtained with silicone resins may be attributable to the intermediate formation of silyl peroxides which are known to have especially good adhesive properties for metals (see the Article "Adhesion Promotion with Silyl Peroxides", by Gordon M. Kline, pp 107-110 of Modern Plastics for May, 1970). The following Example makes use of this property.

#### EXAMPLE 14

2 g of nickel acetoacetone were mixed with 1 g of silicone resin (RTV-11) and 1 g of (75%) 1,1-Di-t-butyl-peroxy-3,3,5-trimethyl cyclohexane, and then heated to about 150° C to provide a yellow-brown non-crystalline, solid. 0.25 g of the solid was dissolved in 50 ml of dichlormethane, and applied to 100 g of finely divided nickel powder (Mond 255). The resultant coated Nickel Powder was dispersed in 110 g of depolymerized rubber, such as that obtained from Hardman Rubber Co. and sold under the trademark HARDMAN DPR 25 7419A to which 17 g of lead peroxide curing agent (#517) was also added. On coating and curing a 0.030 inch thick sheet for 4 hrs. a film was obtained which had a resistance of 10 megohms at low pressure and a resistance of 2 ohms at relatively high manually applied pressure.

Another series of non-peroxy organic compounds adapted to coat and to form electric current passing interfaces with metallic particles are the organic orthotitanates, tetrabutyl titanate, tetrakis (2-ethyl hexyl) 35 orthotitanate, etc., or reaction products thereof. The following Example illustrates this type of composition.

#### EXAMPLE 15

4 g of stannous octoate were mixed with 1 g of tetra-40 butyl titanate whereupon heat evolved. The reaction mixture was dissolved in 50 ml of dichloromethane and the solution mixed with 100 g of carbonyl nickel powder. The solvent was driven off by heating to 110° C. The cooled, coated metal was mixed with 103 g of the 45 silicone RTV-11 of General Electric which had been catalyzed just previously with 0.5 g of dibutyl tin laurate. The mix was cast and cured overnight at room temperature. The resultant film had an electrical resistance of between 10 megohms under low pressure and 50 50 10 ohms under relatively high manually applied pressure.

Conductive or pressure sensitive resistances of an adhesive nature can be made by the process of the invention with matrices of rubber, urethane, silicone and vinyl resins, for example. Such adhesives are useful in forming ground leads (see U.S. Pat. No. 3,762,946, for example), tape circuits, securing terminals, reducing static discharge, shielding layers, security alarm wiring, paste-on circuitry and controls, temporary leads, etc. 60 The following Examples illustrate such an adhesive.

#### EXAMPLE 16

Mond (255) nickel was treated with 1% of the reaction product of nickel octoate and 1,1-di-t-butyl peroxy-3,3,5-trimethylcyclohexane, 55 g of the treated nickel is mixed with 55 g of the adhesive silicone resin composition SR-537 of General Electric. The mix is tacky and

highly conductive. This composition can be marketed as a plastic coating composition.

Many of the above Examples disclose a silicone resin as a matrix material since such resins based on their electrical properties, etc. have advantages. Polyvinyl chloride, however, provides a satisfactory product at a relatively reduced price and the following Example illustrates the manufacture of such a product.

#### EXAMPLE 17

The composition consisted of the following components:

|    |          |                                                 |
|----|----------|-------------------------------------------------|
| 15 | 2 parts  | Dibutyl tin dilaurate                           |
|    | 39 parts | Vinyl chloride resin (GEON 121)                 |
|    | 13 parts | Diocyl phthalate (as plasticizer)               |
|    | 48 parts | Mond 255 nickel powder coated as in Example 14. |

The vinyl resin was blended with the plasticizer to form a powder. The powder was mixed with the coated nickel powder. A cake of the mix was placed between the plates of a hot press at about 168° C and fused. The product had a resistance of 50 megohms under no pressure and 50 ohms at manually applied pressure.

#### EXAMPLE 18

The pressure-resistance graph of FIG. 1 of the drawing was made on the following vinyl-resin matrix material. 100 grams of polyvinyl chloride powder (Geon 121), 60 grams of diocyl phthalate, and 3 grams of dibutyl tin laurate were blended in a high intensity mixer until a uniform pourable vinyl plastisol liquid was obtained which did not separate on standing. In a separate vessel, 40 grams of nickel octoate (6%) and 2 grams of 1,1-di-t-butyl peroxy-3, 3,5-trimethyl cyclohexane were mixed, heated to about 210° C. whereupon reaction occurred; the resultant resin-like solid was dissolved in dichlormethane and applied to 30 grams of Mond nickel 255 to form a 1% coating of the reaction product on the metal. 30 grams of the treated nickel was blended with 30 grams of the vinyl plastisol liquid, degassed, and cast in a Teflon-coated pan to produce a flat flexible sheet slightly over 1 mm thick. The pressure resistance diagram of the drawing was obtained from this material using flat electrodes of 0.200 inch diameter.

Additional experimentation and literature searches have been carried out in an effort to explain the high variation in resistance obtained by this process. These experiments originally fortified my belief in an early hypothesis that the improved results were due to the formation of an incompatible dispersed phase and inhibition of the polymerization of the resin in the region immediately adjacent to the conducting particles. Thus, in Example 1, the inhibitor catalyst, a peroxide, is only present in the mix, whereas improved results were obtained according to Examples 3-5 where an inhibiting catalyst is premixed with the conducting particles, and further improved results were obtained according to Example 6 where the premix of conducting particles and inhibitor is preheated. According to Example 6, the premix of metal includes tin octoate as well as the peroxide inhibitor and there is a reaction between the tin octoate and the peroxide. It should be noted in connection with this hypothesis that the directions for setting the peroxide cured "A and B platinum" type silicone resins of GE's RTV-600 series, state that such resins are not compatible with tin soap cured RTV's and further

state that all molds, etc., which have been used for the latter RTV compounds, must be thoroughly cleaned with soap and water or solvent, then dried and barrier coated before being used for said RTV-600 series. It is also known that particles of colloidal size, such as the conducting particles of the mix, are ordinarily charged and, in suspensions, attract ions of the opposite charge. Thus, in Example I, where the metal particles are not premixed with the inhibiting type of catalyst, a completely cured body is still obtained, possibly because the inhibitor type of catalyst is attracted to the metal particles. Later experiments, such as Example 9, lead me to believe that the inhibitor effect is less important than previously believed. As stated above, there is evidence that a reduction takes place between the benzoyl peroxide and the tin octoate when mixed with the metal particles in Examples 3-8, so that an inhibitor is not necessarily present on the particles added to the resin. Example 9, for example, shows that such a reaction product can be preprepared and thereafter added to the metal conducting particles.

In the product of the invention, particle to particle contact does not appear to be necessary to produce conductivity, and indeed, photomicrographs indicate that particle to particle contact does not always occur, but in practice the coated particles often do come in pressure contact. Thus, particles of relatively low conductivity (see Example 11, for example), coated with a material of relatively low conductivity and embedded in a matrix produce relatively high conductivity on the application of pressure.

One great advantage of this invention is that high conductivities under pressure can be obtained without overloading the elastomeric resin matrix with metal particles. Thus, a product with greater flexibility, greater tensile and compressive strength, and greater durability under repeated pressure cycles is obtained. Also, the product has a lower specific gravity. Thus, the 40 invention has an sp. gr. of around 2.5 whereas a product heavily loaded with metal particles has a sp. gr. of 3.5-4.0. For some applications, the lower sp. gr. can be important.

The material can be made in a complete range of conductivity from 0.01 ohms under pressure to 100 megohms without pressure, for example. The actual conductivity under pressure does depend on the thickness and hardness of the layer and both of these parameters can be readily varied. The conductance produced can be directional or anisotropic, for example, several spaced pairs of pressurizable conductors applied across the thickness of a sheet of the material act independently, i.e., there is little, if any, lateral conductance or interference produced by the neighboring pairs of conducting probes.

The products of the invention produce greater conductivity under pressure than products with the same proportion of metal inclusions, but without the coatings. Also, although no extensive longevity tests have been run on the products of this invention, it is known that they withstand many thousands of applied pressure cycles without substantial deterioration and it is also known that they have greater life under use than commercially available products of the same current carrying capacity. There are several possible explanations for

the improved results obtained with the products of the invention. It will be realized that most available finely divided metal particles are distinctly angular in shape with sharp corners and edges. Applying an adherent coating to such particles rounds off the corners and edges. The applied coating is not rigid or crystalline and instead, is reversibly deformable similar to the elastomer matrix in which the particles are embedded. Although the coating is not as good a conductor as the metal particle itself, the area of contact and number of possible conducting paths is increased considerably when two coated particles come into contact. The result is visualized as similar to that of two balloons being pressed together. This also appears to be similar to the wetting effect noted when a low-conducting liquid is supplied between two conducting bodies which when dry may be brought together, but still do not conduct well because of failure to come into close contact. An additional effect obtained by the coating is that when pressure is applied to the product through two electrodes and then released, the conductivity is abruptly terminated and any tendency towards arcing between sharp particle edges or points is quenched. That is, electrons or holes are spread over the larger surface of the coating rather than being concentrated at the points or edges. It is believed that the short life of some pressure sensitive elastomers containing metallic particles with sharp or angular points or edges can be attributed to microarcing occurring when conducting particles are separated upon releasing the pressure which keeps them in contact. This microarcing results in oxidation and erosion at the arcing points or edges. When not under pressure, the semiconducting coating of the present invention acts as an effective insulator.

An analogous situation has been found in U.S. Pat. No. 3,709,835 of Forster. According to that patent, it was found that the performance of high voltage conductors could be improved by incorporating semi-conducting materials in the insulating coating of the conductors. Column 2, lines 41-47 of said patent read as follows:

"Under low voltage stresses, the semi-conductors act as insulators and conduct no electricity. As the voltage increases to the order of 1.0-100 kilovolts, the semi-conductors begin to conduct electricity, the conductance being a function of the stress applied and increasing as the applied stress increases."

50 Although high voltages are not employed with the pressure sensitive products of this invention, the distances are much closer so that lower voltage differences have the effect of producing a proportionately large dielectric field stress, which results in a conducting or insulating phenomenon similar to that observed by Forster at high voltages.

Also, the coated conducting particles of the invention have a lubricity not possessed by uncoated particles so that said coated particles are more mobile within the elastomer matrix and when moved by pressure being applied to the product, the coated particles do not injure the internal structure of the elastomer.

65 The metallic conducting particles of the present invention can not be compared to the extremely fine carbon particles which are conventionally added to elastomers as the conductive particles. The following table compares the essential properties of typical particles:

|                                            | Surface Area<br>M <sup>2</sup> /g | Sp.<br>Gravity | Particle<br>Shape            | Resistance<br>Microohms/<br>cm | Particle<br>Size |
|--------------------------------------------|-----------------------------------|----------------|------------------------------|--------------------------------|------------------|
| Conductive<br>Carbon<br>Black              | 70.                               | 1.95           | Chain to<br>dendritic        | 1375.0                         | Microns<br>1/70  |
| Carbonyl Ni<br>("Nickel 255")<br>of "Inco" | 0.68                              | 8.9            | Chain<br>and/or<br>Spherical | 6.84                           | Microns<br>2.2   |

Although the metal particles tend to make up for their lower surface area and higher specific gravity (lower vol.%) by their lower resistance, these two types of particles are not really comparable. As already mentioned, the metallic particles, as conventionally added to elastomeric materials for the production of pressure sensitive resistances (except for those coated with noble metals), have oxide coating which increase their resistance, this increase in resistance, due to the oxide layer, is overcome by the present invention.

The dendritic chains of the extremely fine carbon particles which form the conducting path in carbon filled elastomers are much more fragile than the conduction paths formed by the semi-conductor-metal particles of the present invention. The resistance-pressure curves obtained with the metal loaded products of the present invention are substantially the same after many testing cycles, whereas corresponding curves for carbon loaded elastomers change when repeated a number of times. With carbon black, it is not possible to obtain the low values of resistance obtainable with metal, because of its resistance, low specific gravity and the fact that the particles are not physically compactable to produce the lower resistances. With carbon also, there is a higher heating effect resulting from the higher resistivity of the carbon.

Another unusual property of the products of the invention is that, as resistances, they have a positive temperature coefficient. Most resistances have negative temperature coefficients. Carbon, for example, is known for its negative temperature coefficient, and similarly carbon loaded pressure sensitive resistances decrease in resistance as the temperature increases. The materials, therefore, have potential utility as compensating means for resistances with negative temperature coefficients.

I claim:

1. A process for manufacturing a pressure sensitive resistance element of the type comprising a discontinuous phase of conducting particles substantially uniformly distributed in a matrix of a cured polymerizable resin comprising

1. providing a polymerizable, elastomeric resin composition of liquid to pasty consistency which is polymerizable with the aid of a polymerizing catalyst

2. providing finely divided metal conducting particles in a ratio of resin:metal conducting particles of about 100:75 to 100:110 by weight

3. coating the particles with a thin layer of a deformable, electrically semi-conducting compound and mixing the particles with the resin composition, and

4. curing the resultant mix.

2. The process of claim 1 wherein the elastomeric resin is a silicone resin of the type which is cured by a metal soap and wherein the deformable, electrically semi-conducting compound is the reaction product of a peroxy compound with a metal-organic compound.

3. The process of claim 1 wherein the elastomeric resin is a silicone resin of the type which is cured by a

15 peroxy compound and the deformable, semi-conducting compound is the reaction product of a peroxy compound with a metal soap.

4. The process of claim 1 wherein the metal particles are coated by pretreating with a solution of the deformable, semi-conducting compound.

20 5. The process of claim 2 wherein the metal particles are coated by pretreating with a metal-organic compound and then with an aryl peroxy compound to provide a coating of a deformable, semi-conducting compound on the particles.

25 6. An electric resistance element which is sensitive to pressure comprising a substantially discontinuous phase of metallic conducting particles in a matrix of a cured elastomeric resin, said metallic conducting particles having a coating of a deformable, semi-conducting compound thereon, the proportion of resin to metal conducting particles being 100:75 to 100:110 by weight.

30 7. An electric resistance element as claimed in claim 6 wherein the coating on said metal particles comprises a metallo-organic polymer.

35 8. An electric resistance element as claimed in claim 6 wherein the semi-conducting coating on said metal particles comprises a polymer with a series of metal oxygen bonds.

40 9. An electric resistance element as claimed in claim 6 wherein the coating on said metal particle comprises a deformable, semi-conducting non-metallic organic compound.

10. An electric resistance element as claimed in claim 6 wherein the coating on said metal particles comprises a deformable, semi-conducting organic compound which is insoluble in benzene and hexane.

45 11. An electric resistance element as claimed in claim 6 wherein the coating on said metal particles comprises glycerophosphoric acid.

12. The electric resistance element as claimed in claim 6 wherein the metallic conducting particles are coated 50 with a layer of the reaction product of a metal soap and a peroxy compound.

13. The electric resistance element as claimed in claim 6 wherein the metal conducting particles are coated with the reaction product of tin octoate and a peroxy compound.

14. The electric resistance element as claimed in claim 6 wherein the elastomeric resin is a silicone resin.

15. As a composition of matter a flowable composition comprising a continuous phase carrier of resinous insulating material and a dispersed phase of metal conducting particles, said metal particles being coated with a deformable semi-conducting material, said composition being capable of being further congealed whereby it may be coated on regular and irregular surfaces, the proportion of resin to metal particles being 100:75 to 100:110 by weight.

16. An electric resistance element which is sensitive to pressure and which, in a thickness of about  $\frac{1}{8}$  inch has

a resistance decreasing from about 1 megohm to 100 megohms under no pressure to about 100 to about 0.2 ohm under pressure and comprising a substantially discontinuous phase of metal conducting particles of a size of about 0.1 to 44 microns in a matrix of a cured elastomeric resin, the proportion of resin:conducting particles being about 100:75 to 100:110 by weight, said metal particles being coated with the reaction product of a

metal soap and a peroxy compound, said elastomeric resin being incompletely cured at the interfaces of the metal conducting particles and the resin.

17. The electric resistance element as claimed in claim 5 16 wherein the elastomeric resin is a silicone resin.

18. The electric resistance element as claimed in claim 16 wherein the metal soap is tin octoate.

\* \* \* \* \*

10

15

20

25

30

35

40

45

50

55

60

65